

Patented June 24, 1930

1,765,719

# UNITED STATES PATENT OFFICE

WILLIAM J. GAVEN, OF WILKES-BARRE, PENNSYLVANIA, AND MICHAEL FRIED, OF MOUNT VERNON, NEW YORK; MARY E. GAVEN ADMINISTRATRIX OF SAID WILLIAM J. GAVEN, DECEASED

## METHOD OF MAKING COMPOSITION BLANKS

No Drawing. Application filed December 24, 1923. Serial No. 682,580.

This invention relates to an improved method of making composition materials, and more particularly to such composition materials as are supplied to manufacturers of commercial articles, to be formed by means of 5 molds, matrices, or the like into a desired product.

The method heretofore commonly employed in producing such composition materials involves the use of considerable and expensive 10 machinery, the operation of which not infrequently resulted in injury to the workmen or attendants. In carrying out this prior method, the ingredients entering into the 15 composition material, such as clays, pulp, shoddy, mineral material, coloring matter and binder, was first rolled into a mass by means of large revolving heated rolls, requiring from 20 to 45 H. P. for their operation. 20 After the material had been rolled and fused into a heated plastic mass, it was then formed into blanks by means of similar machines of smaller size, and these blanks are finally ground into powder by high power and high 25 speed grinding machines. Such operations are quite laborious and time-consuming, and owing to the great amount of dust arising from the grinding of the materials, and the vapors which are given off in the heating of 30 the mass, are injurious to the health of the workmen.

It is the primary object and purpose of our present invention to provide a new method of making such composition materials, where- 35 by the use of such bulky machinery may be dispensed with, and which method may be carried out in practice with an entire elimination of any injurious effect upon the operator or workman.

More particularly, it is the purpose of our present improvement, to provide such a method, which consists in placing directly upon a non-plastic base a desired amount of the raw, mixed, unrolled, powdered ingredients, consisting of clays, pulp, shoddy, mineral matter, coloring matter, and a suitable binder, and then subjecting such mixed powdered ingredients and the non-plastic base to the action of heat. The resinous or other 45 powdered material is thereby fused, caus- 50 ing the other ingredients to be mechanically held by the binding action, and produces a conglomerate, adherent, homogeneous mass. Under the action of heat, the binder and other materials are 55 also securely fastened and united with the non-plastic base. In some cases we prefer to use a piece of card board or other fibrous material, in which case the said base becomes 60 thoroughly permeated by the plastic mass, so that in effect the powdered ingredients with the binder and the structure of the base become a one piece unit.

As a result of our new method, we produce 65 a composition material which readily lends itself to a variety of treatments. Thus the manufacturer may readily apply to a slab or blank of the composition material an additional or superimposed layer of the powdered ingredients and the binder, or of a plastic mass formed therefrom, and of the same 70 or a different color than the composition blank before placing the latter in the mold, or upon or between matrices, whereby the commercial article is formed or shaped under the 75 action of heat and pressure.

In one embodiment of our present invention, which we have found quite desirable in practice, we provide a base, preferably, though not necessarily, of paper, cloth, or 80 other non-plastic material, which may be of any desired size and shape. Upon one side of this base we then place a sufficient quantity of mixed, dry, powdered ingredients, which are in the raw state, unrolled and ununited 85 with each other. These materials, which include an adhesive binding agent, such as a resinous material, shellac, or the like are evenly spread over the surface of the base, and said base, with the materials thereon, then placed within an oven, or otherwise subjected to the action of heat at substantially 300 to 400° F. for a period of from one to two minutes. This high heat immediately fuses together the 90 powdered resinous particles, whereby the other powdered ingredients are united with each other in a coherent, conglomerate mass; the said binder with the other powdered ingredients also becoming permanently united 95 100

under the action of the same heat with the base.

After the above operation on one side of the base has been completed, it is repeated upon the opposite side thereof, if desired, a similar coat of the raw powdered unfused ingredients being united in a plastic mass, and fixed upon said opposite side of the base in the same manner as above described.

10 We have referred to the use of a base material, such as paper or cloth, but it is to be understood that we may also employ various other non-plastic materials, to which the powdered, raw ingredients formed into a 15 coherent, plastic mass in the manner above described, will adhere or unite.

15 The powdered materials may be placed upon the non-plastic base in various ways, but in order to prevent the admixture of any 20 foreign materials therewith, and also for economical reasons, we prefer to sift the raw, mixed, powdered ingredients upon the surface of the non-plastic base, so that any foreign materials which may by accident find 25 way into the powdered ingredients will be so minute and widely distributed after the sifting operation, that they will not cause any serious damage to the molds, matrices or dies which may be employed in fashioning 30 the blank of composition material into the desired final shape or form of the commercial article, and likewise the article itself will not be defective, and for that reason rejected upon inspection.

35 In order to enable certain shaped blank forms of the composition material to be pressed into the final shape of the commercial article, with a minimum of labor, we may in some cases provide the base with a superimposed member of the same material as the base, but of smaller size, and which part might be of various shapes. This superimposed part is centrally positioned upon the base and the dry, powdered ingredients are 40 then sifted upon the surfaces of said base and the superimposed part, or, if desired, instead of providing such a superimposed part, an additional layer of the dry, powdered material may be applied upon the first applied 45 layer of such material, to cover only a desired portion or section of the base. Thus, in pressing the composition blank to produce the commercial article, the united ingredients will be uniformly spread when said blank 50 is subjected to heat and pressure in the mold or between the dies or matrices. It will be understood that this additional layer forming a raised area may be provided upon either one or both sides of the non-plastic base.

55 Again, in producing phonograph records and the like, the manufacturer may desire that the part of the blank from which the record is formed and upon which the sound record groove is to be inscribed, shall consist of a finer grade of material or shall be of a

different color from the remaining portion of the material. This may be accomplished by applying to that part of the base from which the record surface is to be formed an additional coating of raw, unrolled and unfused powdered ingredients of the desired fineness and quality. This additional layer may be applied either just before subjecting the base with the materials thereon to the action of heat, or when the prepared composition blank is to be formed into the finished article.

From the foregoing description it will be seen that by reason of our new method of forming the composition material we entirely eliminate many of the mechanical operations heretofore required, and thereby reduce the labor involved in the production of such material to a minimum. In addition to the various ways in which a blank formed of such composition material might be used as above explained, it is also apparent that, if desired, the composition blank may be ground or comminuted and pressed into various shapes or forms under the action of heat in suitable molds. Of course, it is also apparent that the composition blanks themselves might be of various forms and sizes, and might be readily built up of a plurality of the formed blanks of the same or different shapes, individually produced in the manner above explained, and then fastened or permanently united with each other in various arrangements; or, if desired, the base sheets of paper or cloth might first be superimposed on each other, and the whole then coated on one or both sides by a plastic composition mass, composed of the mixed, dry, powdered ingredients united under the action of heat in the manner described. It is likewise possible to provide the base with perforations, and when the composition blank formed by fusing the dry, powdered mixed materials upon this perforated base is placed in the mold, the perforated base may be covered with another combination of dry powdered materials united under the action of heat and pressure, and of better quality or of different color from the perforated composition blank.

While it is possible to use various composition materials in carrying out our new method, we preferably employ the following ingredients in substantially the proportions stated:

120  
1 pound of terra alba;  
1 pound of china clay,  
1 pound of wood pulp  
8 pounds of coal dust or culm  
10 pounds of resinous binder with suitable coloring matter.

125  
Of course it is understood that various changes may be made both in the specific ingredients employed and in the relative proportions thereof.

130  
It is to be understood from the foregoing

description, therefore, that the important and essential feature of our new method resides in the application to either one or both sides of a suitable non-plastic base, a coating of unrolled, dry, mixed, powdered raw ingredients, covering either a part or all of the base surface, and then subjecting said base with the composition ingredients thereon to the action of heat at such temperature that the several ingredients are united with each other in a coherent plastic mass, and simultaneously permanently fixed to said base or non-plastic material so as to constitute in effect a component part thereof.

From the foregoing it will be seen that the initial powder contains a resinous binder, as resin, gum, or shellac, and that this is not fused until the heating operation described takes place, when for the first time this resinous binder is subjected to heat. It has been found heretofore, that in all methods heretofore proposed the binder is subjected to heat several times. We have found that each time this is done, the binder has its binding force reduced. We use the binder in its virgin state, and only with one heat and pressure until it is ready for its final pressing, whereby the binder retains its retentive functions throughout.

When the central enlargement in depth is used, either by the powdered material or by the separate non-plastic prepared member, the pressure that is applied, causes the material to be forced or moved radially outwardly and thereby an equal distribution is obtained.

In some cases, it is desirable to place upon the formed blank or base as heretofore described, a sheet of celluloid or celluloid-like material. This can be done on either one or the other sides, or both, if both sides have been treated. To carry out this composite plan, the sheet of celluloid or the like is treated on one side with an adherent cement, and then this cemented portion is placed against the aforesaid base. This celluloid or the like sheet then is cemented to the base. This composite article is then ready to be distributed as a separate article of commerce. The manufacturer then takes this article and subjects it to heat and pressure and molds it to final shape.

Instead of using a sheet of celluloid, or celluloid-like material, a paste or semi-plastic liquid may be prepared, by adding a suitable solvent to the celluloid, and then dipping the formed base into it. Or, it can be applied by a brush to the formed base. It is preferable, however, in the case that celluloid or the like is used, to first equalize the formed base by smoothing it. Then the celluloid-like layer smoothly contacts therewith. This protecting layer maintains the formed base permanently in its initial condition and guards it against the action of the atmosphere, from

moisture, acids, etc. It is also a suitable surface for the impressions of the finished article.

Also, instead of celluloid or celluloid paste or celluloid-like material, a coating of bakelite or condensite or redmonal may be provided in a similar manner, but in this case also the formed base should be smoothed off and a light coating of either one of these three products placed thereon and then subjected to a heat and pressure. We have mentioned bakelite, condensite, redmonal, but of course, any material having a base or binder of formaldehyde or carbolic acid may be used. This also acts as a protecting covering in the manner stated.

This invention may be developed within the scope of the following claim without departing from the essential features of the same and it is desired that the specification be read as being merely illustrative and not in a limiting sense except as necessitated by the prior art.

We claim:

The herein-described method for molding composite plastic and non-plastic articles, which consists in assembling upon a non-plastic base, a coating of unrolled, dry, mixed, powdered, raw ingredients involving a resinous binder in its virgin state, with a central depression in the material whereby the material will be forced to move radially to secure an equal distribution when heated, subjecting said base with the composition ingredients thereon to a single heating for a period of from one to two minutes at a temperature of from 300 to 400° F. whereby the several ingredients are united with each other in a coherent plastic mass and simultaneously permanently fixed to said non-plastic base.

In testimony that we claim the foregoing as our invention, we have signed our names hereto.

WILLIAM J. GAVEN.  
MICHAEL FRIED.

110

115

120

125

130